

# United States Patent [19]

Itou et al.

[11] Patent Number: 4,900,984

[45] Date of Patent: Feb. 13, 1990

[54] CATHODE RAY TUBE WITH ANTISTATIC FILM ON FRONT PANEL

[75] Inventors: Takee Itou, Fukaya; Hidemi Matsuda, Oomiya; Mamory Yoshizako, Machida; Osamu Yagi, Kawasaki, all of Japan

[73] Assignees: Kabushiki Kaisha Toshiba, Kawasaki; Tama Chemicals Co., Ltd., Tokyo, both of Japan

[21] Appl. No.: 187,005

[22] Filed: Apr. 27, 1988

[30] Foreign Application Priority Data

Apr. 28, 1987 [JP] Japan 62-103049

[51] Int. Cl.<sup>4</sup> H01J 29/86

[52] U.S. Cl. 313/479; 313/313

[58] Field of Search 313/479, 477 R, 313; 427/165, 167, 126.2; 358/245, 247

[56] References Cited

U.S. PATENT DOCUMENTS

4,563,612 1/1986 Deal et al. 313/479 X  
4,785,217 11/1988 Matsuda et al. 313/479

FOREIGN PATENT DOCUMENTS

59-96638 6/1984 Japan 313/479  
61-16452 1/1986 Japan  
61-45545 3/1986 Japan

Primary Examiner—Donald J. Yusko

Assistant Examiner—Michael Horabik

Attorney, Agent, or Firm—Cushman, Darby & Cushman

[57] ABSTRACT

A cathode ray tube according to the present invention has a sufficient antistatic property which can be obtained by forming a glass film containing SiO<sub>2</sub> or P<sub>2</sub>O<sub>5</sub> as a main component and a hygroscopic metal salt on the outer surface of its front panel.

5 Claims, 5 Drawing Sheets





FIG. 1  
(PRIOR ART)



F I G. 2



F I G. 3



FIG. 4



F I G. 5

## CATHODE RAY TUBE WITH ANTISTATIC FILM ON FRONT PANEL

### BACKGROUND OF THE INVENTION

#### 1. Field of the Invention

The present invention relates to a cathode ray tube and, more particularly, to a cathode ray tube having an antistatic function.

#### 2. Description of the Related Art

Since the outer surface of a front panel of an envelope of a cathode ray tube has a high surface electric resistance, a static charge accumulates during an operation of the cathode ray tube. This causes inconveniences. For example, dust adheres on the outer surface or an electrical shock is inflicted on a person.

In order to eliminate such inconveniences, Japanese Patent Disclosure No. 61-16452 discloses a cathode ray tube having a transparent thin film composed of a silicate and an inorganic metallic compound of a metal such as platinum, palladium, tin and gold, and formed on the outer surface of its front panel. However, since the silicate in the thin film is not conductive, the surface electric resistance of the thin film cannot be sufficiently decreased. Therefore a sufficient antistatic effect cannot be obtained.

According to the tests performed by the present inventors, when an inorganic metallic compound was not hygroscopic, a thin film was not conductive. When a hygroscopic inorganic metallic compound such as  $PdCl_2$  was added, a low conductivity was obtained. However, when the content of the compound was increased so as to obtain sufficient conductivity, the strength and optical characteristics of the thin film were greatly degraded.

In order to increase the strength of a reflection-free thin film formed on the outer surface of a front panel of an envelope of a cathode ray tube, Japanese Patent Disclosure No. 61-45545 proposes to add an oxide or a hydroxide of a metal such as Ti, Al, Mg, Ca, Zr, Na, and K in the film. However, since it is considered that metal atoms in the oxide or hydroxide are present where Si—O—Si bonds of the skeleton structure of a film-forming material such as  $SiO_2$ , are fragmented as in FIG. 1, the oxide or hydroxide cannot obtain hygroscopicity. Therefore, the resultant film cannot be used as a film required to have conductivity.

### SUMMARY OF THE INVENTION

According to a cathode ray tube according to the present invention, a sufficient antistatic property can be obtained by forming a glass film containing  $SiO_2$  or  $P_2O_5$  as a main component and a hygroscopic metal salt on the outer surface of its front panel.

### BRIEF DESCRIPTION OF THE DRAWINGS

FIG. 1 shows an atomic model of a conventional antistatic glass film for a cathode ray tube;

FIG. 2 shows an atomic model of an antistatic glass film according to an embodiment of the present invention;

FIG. 3 is a graph showing a relationship between the content of an Li salt, and the strength and the resistance of films; and

FIG. 4 is a graph showing a relationship between the content of a Ga salt, and the strength and the resistance of films.

FIG. 5 shows a color picture tube including an antistatic film according to an embodiment of the present invention.

### DETAILED DESCRIPTION OF THE PREFERRED EMBODIMENTS

According to the present invention, as illustrated in FIG. 2, a hygroscopic metallic salt is sealed in the interstices of the skeleton structure (Si—O—Si bonds) of a glass film, and the metal salt absorbs moisture in the air, thereby decreasing the electric resistance of the glass film.

The electric resistance of the glass film can be decreased even if the hygroscopic metal salt is not sealed in the above-described manner. However, it is preferable that the hygroscopic metal salt is sealed in the above-described manner so as to be firmly fixed in the glass film. In order to seal the metal salt in the above-described manner, its size must be small. If the size of the metal salt is excessively large, it causes the glass skeleton to break, and the strength of the film is thereby decreased. Consequently, the metal salt cannot be added in an amount necessary to obtain a sufficient conductivity.

The thickness of a glass film is preferably 0.05 to 1  $\mu m$ . If it is smaller than 0.05  $\mu m$ , the electric resistance of the film cannot be stabilized. On the other hand, if it is larger than 1  $\mu m$ , it becomes difficult to uniformly form the film, thereby causing the focus of an image to blur.

Table 1 shows the strength of each film when a corresponding metal salt is contained in an amount sufficient for obtaining a film resistance of  $5 \times 10^{10} \Omega/cm^2$ . The film strength was determined by a rubbing test of a corresponding film using an eraser, i.e., Lion No 50-30 (trademark) to which a load of  $200 g/cm^2$  was applied. The film strength was represented by the number of times reciprocal rubbing motions could be repeatedly applied until the film peeled. It is found from Table 1 that the strength of the film tends to increase as the atomic number of metallic elements in a metal salt is decreased. Practical metal salts (having strengths of 60 or more times) are those containing metallic elements having atomic numbers which are smaller than that of Ga (31). Although the metal salts are represented as anhydrous salts in Table 1, some of them can be hydrous salts.

TABLE 1

| Metallic Element | Atomic Number | Film Strength (number of times)    |                             |                       |
|------------------|---------------|------------------------------------|-----------------------------|-----------------------|
|                  |               | (Chloride)                         | (Nitrate)                   | (Sulfate)             |
| Li               | 3             | 100 or more<br>( $LiCl$ )          | 100 or more<br>( $LiNO_3$ ) | —                     |
| Be               | 4             | 100 or more<br>( $BeCl_2$ )        | —                           | —                     |
| Ca               | 20            | 90 ( $CaCl_2$ )                    | 85 ( $Ca(NO_3)_2$ )         | —                     |
| Sc               | 21            | 70 ( $ScCl_3$ )                    | 65 ( $Sc(NO_3)_3$ )         | —                     |
| Mn               | 25            | 80 ( $MnCl_2$ )                    | —                           | —                     |
| Fe               | 26            | 75 ( $FeCl_2$ )<br>65 ( $FeCl_3$ ) | 60 ( $Fe(NO_3)_3$ )         | 60 ( $Fe(SO_4)_3$ )   |
| Ni               | 28            | 70 ( $NiCl_2$ )                    | 65 ( $Fe(NO_3)_2$ )         | 70 ( $NiSO_4$ )       |
| Cu               | 29            | 70 ( $CuCl_2$ )                    | 65 ( $Cu(NO_3)_2$ )         | —                     |
| Zn               | 30            | 70 ( $ZnCl_2$ )                    | —                           | —                     |
| Ga               | 31            | 65 ( $GaCl_3$ )                    | 65 ( $Ga(NO_3)_3$ )         | 60 ( $Ga_2(SO_4)_3$ ) |
| Rb               | 37            | —                                  | 55 ( $RbNO_3$ )             | —                     |
| Sr               | 38            | 50 ( $SrCl_2$ )                    | —                           | —                     |
| Mo               | 42            | 40 ( $MoCl_5$ )                    | —                           | —                     |
| Pd               | 46            | 50 ( $PdCl_2$ )                    | 45 ( $Pd(NO_3)_2$ )         | 45 ( $PdSO_4$ )       |

TABLE 1-continued

| Metallic Element | Atomic Number | Film Strength (number of times) |           |           |
|------------------|---------------|---------------------------------|-----------|-----------|
|                  |               | (Chloride)                      | (Nitrate) | (Sulfate) |
| Au               | 79            | 30 (AuCl <sub>3</sub> )         | —         | —         |

Hygroscopic salts having metallic elements with atomic numbers of 31 or less are e.g., LiCl, LiBr, LiI, LiNO<sub>3</sub>, BeF<sub>2</sub>, BeCl<sub>2</sub>, BeCl<sub>2</sub>.4H<sub>2</sub>O, BeBr<sub>2</sub>, NaI, NaI.2H<sub>2</sub>O, NaNO<sub>3</sub>, MgCl<sub>2</sub>, MgCl<sub>2</sub>.6H<sub>2</sub>O, MgBr<sub>2</sub>, MgBr<sub>2</sub>.6H<sub>2</sub>O, MgI<sub>2</sub>, MgI<sub>2</sub>.8H<sub>2</sub>O, Mg(NO<sub>3</sub>)<sub>2</sub>.6H<sub>2</sub>O, AlCl<sub>3</sub>, AlBr<sub>3</sub>, AlBr<sub>3</sub>.6H<sub>2</sub>O, AlI<sub>3</sub>, KF, KF.2H<sub>2</sub>O, KBr, CaCl<sub>2</sub>, CaCl<sub>2</sub>.H<sub>2</sub>O, CaCl<sub>2</sub>.2H<sub>2</sub>O, CaCl<sub>2</sub>.6H<sub>2</sub>O, CaBr<sub>2</sub>, CaBr<sub>2</sub>.6H<sub>2</sub>O, CaI<sub>2</sub>, CaI<sub>2</sub>.6H<sub>2</sub>O, Ca(NO<sub>3</sub>)<sub>2</sub>, Ca(NO<sub>3</sub>)<sub>2</sub>.4H<sub>2</sub>O, ScCl<sub>3</sub>, ScBr<sub>3</sub>, Sc(NO<sub>3</sub>)<sub>3</sub>, TiCl<sub>3</sub>, TiBr<sub>4</sub>, Ti(SO<sub>4</sub>)<sub>2</sub>, VF<sub>4</sub>, VCl<sub>2</sub>, VCl<sub>3</sub>, VBr<sub>3</sub>, CrCl<sub>2</sub>, CrCl<sub>3</sub>, CrI<sub>2</sub>, MnCl<sub>2</sub>, MnCl<sub>2</sub>.4H<sub>2</sub>O, MnBr<sub>2</sub>, MnI<sub>2</sub>, MnI<sub>2</sub>.4H<sub>2</sub>O, FeCl<sub>2</sub>, FeCl<sub>2</sub>.4H<sub>2</sub>O, FeCl<sub>3</sub>.6H<sub>2</sub>O, FeBr<sub>2</sub>.6H<sub>2</sub>O, FeBr<sub>3</sub>, FeI<sub>2</sub>, FeI<sub>2</sub>.4H<sub>2</sub>O, Fe(NO<sub>3</sub>)<sub>3</sub>.9H<sub>2</sub>O, Fe<sub>2</sub>(SO<sub>4</sub>)<sub>3</sub>.9H<sub>2</sub>O, CoCl<sub>2</sub>, CoBr<sub>2</sub>, CoBr<sub>2</sub>.6H<sub>2</sub>O, CoI<sub>2</sub>, CoI<sub>2</sub>.2H<sub>2</sub>O, CoI<sub>2</sub>.6H<sub>2</sub>O, Co(NO<sub>3</sub>)<sub>2</sub>.6H<sub>2</sub>O, NiCl<sub>2</sub>, NiCl<sub>2</sub>.6H<sub>2</sub>O, NiBr<sub>2</sub>, NiI<sub>2</sub>, Ni(NO<sub>3</sub>)<sub>2</sub>.6H<sub>2</sub>O, NiSO<sub>4</sub>, CuCl<sub>2</sub>, CuCl<sub>2</sub>.2H<sub>2</sub>O, CuBr<sub>2</sub>, Cu(NO<sub>3</sub>)<sub>2</sub>.3H<sub>2</sub>O, Cu(NO<sub>3</sub>)<sub>2</sub>.6H<sub>2</sub>O, ZnC<sub>3</sub>S<sub>2</sub>, ZnBr<sub>2</sub>, GaCl<sub>3</sub>, GaBr<sub>3</sub>, Ga(NO<sub>3</sub>)<sub>3</sub>.xH<sub>2</sub>O, Ga<sub>2</sub>(SO<sub>4</sub>)<sub>3</sub>, and Ga<sub>2</sub>(SO<sub>4</sub>)<sub>3</sub>.18H<sub>2</sub>O.

For some unknown reason, as the atomic number of metallic elements in a salt is reduced, the electric resistance of a film is further decreased and such a salt of metal with a small atomic number can provide an antistatic effect with a small content. Generally, when the content of a metal salt exceeds a given amount (10 wt % with respect to the total weight of the glass film), the strength of a film is abruptly decreased. When a film resistance of  $5 \times 10^{10} \Omega/\text{cm}^2$  is to be obtained, a content of a metal salt up to 10 wt % is sufficient if a salt of a metal with an atomic number of 31 or less is used. If a salt of a metal with an atomic number greater than 31 is used, a content of 10 wt % or more is required, resulting in a decreased film strength.

A material constituting a skeleton of a glass film is SiO<sub>2</sub>, P<sub>2</sub>O<sub>5</sub>, or a mixture thereof. These substances are preferably in the form of an alcoholate. In order to improve the film strength, B, Zr, Ti, Fe, Al, V, or the like may be contained therein.

A film according to the present invention can be obtained by dissolving one of the above-described hygroscopic metal salts in an alcoholate of the skeleton component, and coating the resultant solution on a cathode ray tube by means of a spray method, a spin method, a dip method, or the like.

FIG. 3 shows a relationship between the contents of a metal salt with respect to a skeleton component (main component) such as SiO<sub>2</sub>, and the strength and electric resistance of a corresponding film, when LiNO<sub>3</sub>, which exhibits the largest antistatic effect, is used. When LiCl is used, the same figure is obtained.

It is apparent from FIG. 3 that a content of 10 wt % or less is preferable when considering the film strength, and 0.001 wt % or more is preferable when considering the resistance of the film. FIG. 4 shows a case when Ga(NO<sub>3</sub>)<sub>3</sub> is used. In this case, an added amount of 10 wt. % or less is preferable in consideration of strength, and 5 wt. % or more is preferable in consideration of the resistance of the film. The same figure is obtained when GaCl<sub>3</sub> or Ga(SO<sub>4</sub>)<sub>3</sub> is used.

A more preferable range varies depending on the solubility of a metal salt to water and an alcohol (a

solvent for preparing a coating solution), the molecular weight, and the hygroscopicity of a metal salt.

When a glass film is formed from the solution containing a hygroscopic metal salt and a polysiloxane alcoholate of Si, the content of the hygroscopic metal salt in a glass film becomes 1/10 that of the solution since the volume of the film is decreased through evaporation of a solvent or dehydrating condensation reaction during the formation of the film (the production of SiO<sub>2</sub>), and hence the hygroscopic metal salt caused to separate from the film. Therefore, in order to form a glass film containing 0.001 to 10 wt % hygroscopic metal salt with respect to a main component, the hygroscopic metal salt must be contained in a glass solution in an amount of 0.01 to 100 wt % with respect to SiO<sub>2</sub> stoichiometrically produced from polysiloxane or alcoholate of Si.

According to the present invention, the adhesion strength of a film with respect to a cathode ray tube is improved. Although the reason for this is not clear, it may be presumed that a dense film is formed because the metal salt is filled in the interstices of a skeleton component.

#### EXAMPLE 1

A coating solution having the following composition was prepared.

ethyl silicate . . . 5 wt. %  
nitric acid . . . 3 wt %  
water . . . 2 wt %  
lithium nitrate . . . 0.5 wt %  
isopropyl alcohol . . . balance

This solution was coated on a face plate 2 of a cathode ray tube 1 by means of a spin method and baked at 115°C. for ten minutes to form an antistatic film having an average thickness of 0.1 μm as shown in FIG. 1. The amount of the metal salt (lithium nitrate) was 3.03% with respect to the total weight of the film. The antistatic film exhibited a resistance of  $5 \times 10^8 \Omega/\text{cm}^2$  at 20°C. and 40% RH.

As a comparative example, a film without lithium nitrate, and a film containing 0.01 wt % (with respect to the film weight) of SnCl<sub>4</sub> using a lithium stabilized silicon sol disclosed in Japanese Patent Disclosure 61-16452 in place of lithium nitrate were formed to have the same thickness as that in Example 1. The resistances of these films were  $5 \times 10^{11}$  and  $2 \times 10^{11} \Omega/\text{cm}^2$ , respectively.

In the rubbing tests described above, the film on a cathode ray tube according to the present invention exhibited a strength which could withstand a 100 times more of eraser rubbing and was superior in resistance to wear as compared to the film in the comparative example, which exhibited a strength which could withstand a rubbing of 80 times.

#### EXAMPLE 2

A film was formed following the same procedure as in Example 1 except that sodium nitrate was used in place of lithium nitrate. Although the film exhibited a resistance of  $9 \times 10^9 \Omega/\text{cm}^2$ , the antistatic effect was sufficient for practical use.

#### EXAMPLE 3

A solution having the same composition as that in Example 1 was used and coated on a faceplate of a cathode ray tube by means of the spray method. Then,

solution was baked at 150° C. for 30 minutes to form a film. The resistance of the film was  $1 \times 10^9 \Omega/\text{cm}^2$ . In this case the film exhibited a flicker prevention effect. When the films in the comparative examples were formed by means of the spray method, the flicker prevention effect was also obtained in each film. However, their resistances were  $10^{12} \Omega/\text{cm}^2$  or more, and  $1 \times 10^{11} \Omega/\text{cm}^2$ , respectively. Thus, the prominent anti-static effect of the present invention was demonstrated.

What is claimed is:

1. A cathode ray tube comprising:  
an envelope having a front panel; and  
a glass film formed on said front panel and containing  
 $\text{SiO}_2$  or  $\text{P}_2\text{O}_5$  as a main component and a hygroscopic metal salt sealed in the interstices of the 15  
skeleton structure of said glass film.
2. A cathode ray tube according to claim 1, wherein  
said hygroscopic metal salt is a salt of a metallic element  
having an atomic number of 31 or less.

10

20

3. A cathode ray tube according to claim 1, wherein  
said hygroscopic metal salt is contained in said glass  
film in an amount of 0.001 to 10% by weight with respect to said main component.

4. A glass solution for an antistatic film of a cathode ray tube comprising:  
a polysiloxane or alcoholate of Si; and  
a hygroscopic metal salt in an amount of 0.01 to 100% by weight with respect to  $\text{SiO}_2$  stoichiometrically produced from said polysiloxane or alcoholate of Si.

5. A cathode ray tube comprising:  
an envelope having a front panel; and  
a glass film formed on said front panel and containing  
 $\text{SiO}_2$  or  $\text{P}_2\text{O}_5$  as a main component and a hygroscopic metal salt of a metallic element having an atomic number of 31 or less sealed in the interstices of the skeleton structure of said glass film.

\* \* \* \* \*

25

30

35

40

45

50

55

60

65